

## UNITED STATES PATENT OFFICE

2,634,205

LOW ALLOY STEEL OF HIGH YIELD  
STRENGTH

Peter Payson, New York, N. Y., and Alvin E. Nehrenberg, Bloomfield, N. J., assignors to Crucible Steel Company of America, New York, N. Y., a corporation of New Jersey

No Drawing. Application August 17, 1950,  
Serial No. 180,090

3 Claims. (Cl. 75—125)

## 1

This invention pertains to a relatively low alloy steel of exceptionally high yield strength.

It is an object of the invention to provide a readily weldable low carbon, low alloy steel which in the as rolled, or normalized, condition has a minimum yield strength (at 0.2% offset) of about 90,000 p. s. i. There are many high strength, low alloy structural steels being marketed at present which as rolled have nominal yield strengths of about 50,000 p. s. i. and a few of these in the as rolled condition have yield strengths as high as 70,000 p. s. i. but none so far as we know has the desired combination of good weldability, relatively low alloy content, and yield strength of 90,000 p. s. i. or more, as provided by the steel of our invention. It is obvious that higher yield strength in the steel makes for lighter weight construction which is especially desirable for mobile equipment such as railroad cars, automobiles, buses, trucks, aircraft, steam shovels, derrick booms, gun carriages, and the like, as well as for heavy stationary structures such as bridges and hangars in which a considerable part of the steel used is necessary to support the weight of the steel itself.

Ordinary low carbon steel, as cooled in air has a structure of ferrite and pearlite which is quite weak. Furthermore, the ordinary low carbon steel cannot be strengthened very much even by heat treatment because of the very rapid trans-

alloying elements, and that it is preferable to use a number of alloying elements instead of one or two. The common alloying elements which are most effective for increasing hardenability are manganese, molybdenum and chromium, in that order. Since manganese is the most effective and least expensive of these elements we use a minimum of 1.0% of manganese in our steel and may use as much as 2.0% manganese. Since molybdenum is much more expensive than manganese we use a smaller amount from about .05 to .60% of this element in our steel. Chromium is used up to about 1.2%, although generally we limit this element to about 0.80%.

As is well known, it is desirable that the high strength low alloy steels should be more rust resistant than ordinary carbon steel and for this purpose we add about 0.20 to 0.60% copper to our steel.

In order to assure good weldability in the steel of our invention, we limit the carbon to 0.15% maximum and to assure good strength we set the carbon minimum at .05%, although we generally aim to get between .08 and .15% carbon in the steel.

Now we have discovered that a steel as outlined above but with further additions of silicon and nickel has a very high yield strength in the as rolled, or normalized, or stress relieved conditions as shown by the data below.

TABLE I  
Effect of silicon on yield strength and ductility

| Bar  | Analysis, Percent |      |      |      |      |      |     |     |     | As Air Cooled from<br>1725/1750° F., in<br>1/2" rd. |      |
|------|-------------------|------|------|------|------|------|-----|-----|-----|-----------------------------------------------------|------|
|      | C                 | Mn   | P    | S    | Si   | Ni   | Cr  | Mo  | Cu  |                                                     |      |
| 5462 | .09               | 1.37 | .008 | .023 | .38  | 1.86 | .75 | .23 | .38 | 81,000                                              | 19.1 |
| 5463 | .09               | 1.37 | .008 | .024 | .91  | 1.76 | .73 | .23 | .39 | 90,000                                              | 19.4 |
| 5163 | .14               | 1.18 | .010 | .019 | .84  | 1.86 | .34 | .22 | .47 | 79,000                                              | 19.5 |
| 5257 | .14               | 1.20 | .009 | .019 | 1.61 | 1.80 | .45 | .36 | .38 | 100,000                                             | 17.7 |

formation of the austenite of such steel during a water quench. For example, Sisco in "Alloys of Iron and Carbon," page 195, shows that low carbon steel as water quenched and tempered at 1000° F. has a yield strength of only 62,000 p. s. i.

It is well known that the transformation of austenite can be retarded, that is, the hardenability of the steel can be increased, by use of

It will be noted that in the first two steels of Table I all elements are the same except silicon and the steel with 0.91% silicon has a much better yield strength than the one with only 0.38 silicon. Also, in the last two steels of this group all elements are nearly the same except silicon, and of these two, the one with 1.61 silicon has a very much better yield strength than the steel

with 0.84 silicon. On the basis of these data we set the silicon limits for our steel at 0.90 to 2.0%.

The effect of nickel is shown in Table II.

steels which are nearly alike except for nickel, bar 5460 with 1.03% Ni has a yield strength of only 70,000 p. s. i. whereas bar 5461 with 1.77%

TABLE II  
*Effect of nickel on yield strength and ductility*

| Bar       | Analysis, Percent |      |      |      |      |      |      |     |     | As Air Cooled from 1725/1750° F., in $\frac{1}{2}''$ rd. |                          |
|-----------|-------------------|------|------|------|------|------|------|-----|-----|----------------------------------------------------------|--------------------------|
|           | C                 | Mn   | P    | S    | Si   | Ni   | Cr   | Mo  | Cu  | 0.2% Yield, p. s. i.                                     | Elong. in 2 in., percent |
| 5457..... | .09               | 1.31 | .008 | .023 | 1.54 | .09  | 1.00 | .25 | .40 | 55,500                                                   | 23.7                     |
| 5458..... | .09               | 1.41 | .008 | .021 | 1.61 | .43  | .82  | .27 | .41 | 76,500                                                   | 19.4                     |
| 5459..... | .08               | 1.40 | .008 | .023 | 1.44 | 1.01 | .80  | .26 | .38 | 75,000                                                   | 22.0                     |
| 5259..... | .14               | 1.19 | .008 | .018 | 1.19 | 2.17 | .88  | .25 | .37 | 103,500                                                  | 17.8                     |
| 5460..... | .10               | 1.44 | .008 | .022 | 1.62 | 1.03 | .82  | .02 | .40 | 70,000                                                   | 20.6                     |
| 5461..... | .10               | 1.55 | .009 | .022 | 1.61 | 1.77 | .79  | .08 | .39 | 97,000                                                   | 19.2                     |

It will be noted that the first steel in the group in Table II containing high Mn, high Si, high Cr, and Mo and Cu, but with very little Ni, has a relatively low yield strength, about equivalent to that found in commercial high strength low alloy steels. The next steel bar 5458 with about 0.5% Ni has a much higher yield strength, but the third

Ni has the very high yield strength of 97,000 p. s. i. with over 19% elongation. On the basis of these results, we set the nickel limits for our steel at 1.50% to 2.5%.

As an illustration of other steels which come within the composition limits of our invention we list those shown in Table III.

TABLE III  
*Additional examples of steels of this invention*

| Bar       | Analysis, Percent |      |      |      |      |      |      |     |     | As Air Cooled from 1725/1750° F., in $\frac{1}{2}''$ rd. |                          |
|-----------|-------------------|------|------|------|------|------|------|-----|-----|----------------------------------------------------------|--------------------------|
|           | C                 | Mn   | P    | S    | Si   | Ni   | Cr   | Mo  | Cu  | 0.2% Yield, p. s. i.                                     | Elong. in 2 in., percent |
| 5253..... | .10               | 1.23 | .008 | .019 | 1.44 | 1.86 | .47  | .44 | .37 | 95,000                                                   | 18.0                     |
| 5254..... | .13               | 1.22 | .009 | .022 | 1.59 | 1.75 | .47  | .43 | .36 | 100,500                                                  | 17.6                     |
| 5252..... | .12               | 1.16 | .009 | .023 | 1.48 | 1.74 | 1.06 | .42 | .61 | 113,000                                                  | 17.1                     |
| 2141..... | .14               | 1.25 | .011 | .016 | 1.59 | 1.86 | .14  | .55 | .59 | 102,000                                                  | 16.0                     |

steel with 1.0% Ni has about the same yield strength as the second. However, the fourth steel, bar 5259, with 2.17% Ni has the exceedingly

Tensile data to show the effect of stress relieving after normalizing on steels of this invention are shown in Table IV.

TABLE IV

*Effect of stress relieving on steels of this invention as normalized  $\frac{1}{8}$  in. sq. section from 1750° F. then stress relieved at 1100° F. for 1 hour*

| Bar       | C   | Mn   | Si   | Ni   | Cr   | Mo  | Cu  |
|-----------|-----|------|------|------|------|-----|-----|
| 5252..... | .12 | 1.16 | 1.48 | 1.74 | 1.06 | .42 | .61 |
| 5253..... | .10 | 1.23 | 1.44 | 1.86 | .47  | .44 | .37 |
| 5461..... | .10 | 1.55 | 1.01 | 1.77 | .79  | .08 | .39 |

|                                | Bar 5252 |             | Bar 5253 |             | Bar 5461 |             |
|--------------------------------|----------|-------------|----------|-------------|----------|-------------|
|                                | Norm.    | Stress Rel. | Norm.    | Stress Rel. | Norm.    | Stress Rel. |
| 0.2% Yield Str., p. s. i.....  | 122,000  | 118,000     | 102,000  | 100,000     | 96,000   | 95,000      |
| Tensile Strength, p. s. i..... | 169,000  | 122,000     | 148,000  | 122,000     | 146,500  | 109,000     |
| Elong. in 2 in., Percent.....  | 18.2     | 18.5        | 19.0     | 17.4        | 19.4     | 24.2        |
| Red. Area, Percent.....        | 58.6     | 56.8        | 56.0     | 61.1        | 54.4     | 64.1        |
| Rockwell C Hardness.....       | 35.5     | 29.5        | 31.5     | 25          | 32.5     | 21.5        |

high yield strength for normalized steel of 103,500 p. s. i. and this together with an elongation value of 17.8%. Again in a comparison of the last two

Data on sheet stock of several thicknesses tested both as rolled and after a stress relief treatment of 1 hour at 1100° F. are given below.

*Mechanical properties of sheets of several sizes of steel of this invention tested both as rolled and as stress relieved at 1100° F. for 1 hour*

| C   | Mn   | Si   | Ni   | Cr   | Mo  | Cu  |
|-----|------|------|------|------|-----|-----|
| .12 | 1.25 | 1.26 | 1.83 | 1.01 | .10 | .45 |

|                                | 1/16 in. thick |                | 1/8 in. thick |                | 1/4 in. thick |                |
|--------------------------------|----------------|----------------|---------------|----------------|---------------|----------------|
|                                | As<br>Rolled   | Stress<br>Rel. | As<br>Rolled  | Stress<br>Rel. | As<br>Rolled  | Stress<br>Rel. |
| 0.2% Yield Str., p. s. i. .... | 123,000        | 113,500        | 154,000       | 138,000        | 115,000       | 120,000        |
| Tensile Str., p. s. i. ....    | 160,000        | 139,000        | 178,000       | 148,000        | 165,000       | 137,000        |
| Elong. in 2 in., Percent ....  | 12.5           | 11             | 11            | 12.5           | 13            | 16             |
| Red. Area, Percent ....        | 18             | 35             | 38            | 41             | 25            | 47             |

To summarize, the invention comprises a low alloy, high strength steel characterized in having in the as rolled and normalized conditions, in sections up to about one inch, a minimum yield strength at 0.2% offset, of 90,000 pounds per square inch, said steel comprising, in accordance with a broad range of analysis, about: 0.05 to 0.15% carbon; 1 to 2% manganese; 0.9 to 2% silicon; 1.5 to 2.5% nickel; chromium up to 1.2%; 0.05 to 0.6% molybdenum; 0.2 to 0.6% copper; up to 0.05% maximum, each of sulphur and phosphorus; and the balance substantially all iron, i. e., iron except for the usual impurities within commercial tolerances.

A more preferred range of analysis comprises about: 0.08 to 0.15% carbon; 1.15 to 1.6% manganese; 1.2 to 1.8% silicon; 1.6 to 2.1% nickel; 0.5 to 1% chromium; 0.08 to 0.15% molybdenum; 0.25 to 0.5% copper; sulphur and phosphorus not to exceed 0.05% each, and the balance substantially all iron.

We claim:

1. A low alloy, high strength steel characterized in having in the as rolled and normalized conditions, in sections up to about one inch, a minimum yield strength at 0.2% offset of 90,000 pounds per square inch, said steel comprising about: 0.05 to 0.15% carbon; 1 to 2% manganese; 0.9 to 2% silicon; 1.5 to 2.5% nickel; 0.14 to 1.2% chromium; 0.05 to 0.6% molybdenum; 0.2 to 0.6% copper; up to 0.05% maximum, each of sulphur and phosphorus; and the balance iron.

2. A low alloy, high strength steel characterized in having in the as rolled and normalized conditions, in sections up to about one inch, a minimum yield strength at 0.2% offset of 90,000 pounds per square inch, said steel comprising

about: 0.08 to 0.15% carbon; 1.15 to 1.6% manganese; 1.2 to 1.8% silicon; 1.6 to 2.1% nickel; 0.5 to 1% chromium; 0.08 to 0.15% molybdenum; 0.25 to 0.5% copper; up to 0.05% maximum, each of sulphur and phosphorus; and the balance iron.

3. A low alloy, high strength steel characterized in having in the as rolled and normalized conditions, in sections up to about one inch, a minimum yield strength at 0.2% offset of 90,000 pounds per square inch, said steel comprising about: 0.05 to 0.15% carbon; 1 to 2% manganese; 0.9 to 2% silicon; 1.5 to 2.5% nickel; 0.5 to 1.2% chromium; 0.05 to 0.6% molybdenum; 0.2 to 0.6% copper; up to 0.05% maximum, each of sulphur and phosphorus; and the balance iron.

PETER PAYSON.

ALVIN E. NEHRENBURG.

#### REFERENCES CITED

The following references are of record in the file of this patent:

#### UNITED STATES PATENTS

Number Name Date  
45 2,447,089 Payson, et al. Aug. 17, 1948

#### FOREIGN PATENTS

Number Country Date  
50 673,465 Germany Mar. 22, 1939

#### OTHER REFERENCES

Alloys of Iron and Copper, page 168. Edited by Gregg and Daniloff. Published in 1934 by the McGraw-Hill Book Co., New York.

55 Metal Progress, July 1935, page 29. Published by the American Society for Metals, Cleveland, Ohio.